

## UNITED STATES PATENT OFFICE

ELMER W. ADAMS, OF HAMMOND, INDIANA, ASSIGNOR TO STANDARD OIL COMPANY, OF WHITING, INDIANA, A CORPORATION OF INDIANA

## SULPHURIZED OILS

No Drawing.

Application filed August 8, 1929. Serial No. 384,503.

The present invention relates to improvements in sulphurized oils, such oils being useful for the lubrication of cutting tools and the like.

5 The present invention has to do more particularly with sulphurized cutting oils consisting principally of hydrocarbon oils and free from fatty oils. In the production of such oils in the past, employing high grade 10 lubricating oil fractions, such as lubricant distillates from Mid-Continent and Pennsylvania crudes as a base, it has been possible to secure a product containing only up to about 3% total sulfur, and such oils, when 15 so prepared as to contain above 2% of total sulfur, are extremely dark, being almost black. As a result their use makes it substantially impossible to follow closely the work of a cutting tool. Furthermore, by 20 producing the oils in the manner hitherto employed, if a light colored cutting oil is desired, free from animal or fatty oils, it must be prepared of so low a sulfur content as to markedly reduce its value as a cutting 25 lubricant.

Although the value of the oil as a cutting lubricant has hitherto been attributed to the additional sulfur incorporated into the oil by heating elemental sulfur therewith, it 30 has now been found that by incorporating sulfur into a hydrocarbon stock having initially a high sulfur content, say in excess of 0.75%, an additional quantity of sulfur can be incorporated so that sulphurized cutting oils containing substantially in excess 35 of 3% total sulfur can be secured, and relatively light colored products containing as high as 2½ to 3% sulfur can be prepared. It has furthermore been found that, on incorporation of additional elemental sulfur 40 into such stocks having initially high sulfur content, the total sulfur is of effective value in cutting lubrication.

The optimum condition for incorporating 45 sulfur into such mineral oils, has been found to be the heating of a slight excess of sulfur with the desired lubricating oil fraction at temperatures 300 to 350° F. for a period of 3 to 5 hours. For example, by heating a 50 coastal distillate oil of 200 sec. viscosity at

100° F. and 2.5% sulfur content with sulfur in the proportion of 100 gallons of oil to 39 lbs. of sulfur to 350 to 360° F. for 5 hours with agitation by steam, and straining out the sludge and unused sulfur, a product 55 containing about 5.3% sulfur has been produced. A similar treatment of a distillate oil having an initial sulfur content of about 2.3% yielded a product having a total sulfur content of 5%.

When a light colored product of high sulfur content is desired, a treated high-sulfur lubricant fraction may be employed. Such products, derived, for example, by the ordinary sulfuric acid treatment and clay 65 filtration of high sulfur lubricant fractions, may contain from .75% sulfur up, and products containing as high as 2.5 to 3% sulfur and having a color of 3½ to 6 N. P. A. can be secured. Thus by heating 70 a refined hydrocarbon distillate having a viscosity of 110 sec. at 100° F. and a sulfur content of 1.3% with 2% of sulfur at a temperature of 300 to 320° F. for 3 hours, a product having a 2.8% sulfur and a color of 75 4-4½ N. P. A. is secured. A product of similar sulfur content, produced by the methods and from the stocks hitherto employed, would be practically black, and would have no better value as a cutting lubricant than the relatively light product produced in accordance with the present invention. It appears that, after the incorporation of the additional sulfur, the original sulfur as well as the additional sulfur function to improve the value of the oil as a cutting lubricant.

I claim:

1. The method of producing a sulphurized cutting oil which comprises incorporating 90 into hydrocarbon oil free from fatty oil and containing initially at least 0.75% sulfur, additional sulfur sufficient to bring the total sulfur content of the oil to at least 2%.

2. The method of producing a light-colored 95 sulphurized cutting oil which comprises heating a treated hydrocarbon oil distillate free from fatty oil and containing initially at least 0.75% sulfur, with additional sulfur sufficient to bring the total sulfur to 2% to 100

3%, said heating being at a temperature of 300 to 350° F.

3. The method of producing a sulphurized cutting oil which comprises heating a hydrocarbon oil distillate free from fatty oil and containing at least 0.75% sulfur, with additional sulfur to bring the total sulfur content of the oil to at least 2%, the heating being at a temperature of 300 to 350° F.

10 4. A sulphurized cutting oil consisting principally of hydrocarbon oil having an initial sulfur content of at least 0.75% and free from fatty oil, said cutting oil containing 2-3% sulfur and having a color not darker than 6 N. P. A.

15 5. The method of producing a sulphurized cutting oil having a color not darker than 6 N. P. A. and having a total sulfur content of at least 2% which comprises incorporating into hydrocarbon oil free from fatty oil and containing initially at least 0.75% sulfur, additional sulfur sufficient to bring the total sulfur content of the oil to at least 2%.

20 6. The method of producing a sulphurized cutting oil having a color not darker than 6 N. P. A. and having a total sulfur content as high as 3% which comprises heating a treated hydrocarbon oil distillate free from fatty oil and containing initially at least 0.75% sulfur, with additional sulfur sufficient to bring the total sulfur content up to the desired proportion, said heating being at a temperature of 300 to 350° F.

25 7. A sulphurized cutting oil consisting principally of hydrocarbon oil having an initial sulfur content of at least 0.75% and containing from 1.25% to 2.25% of added sulfur, said cutting oil being free from fatty oil and having a color not darker than 6 N. P. A.

30 8. A sulphurized cutting oil containing hydrocarbon mineral oil having a total sulfur content in excess of 3% of the hydrocarbon oil and including at least 0.75% initial sulfur content of the hydrocarbon oil and the remaining sulfur combined directly with the hydrocarbon oil.

ELMER W. ADAMS.